# EUROPEAN PATENT SPECIFICATION

(11) **EP 4 004 955 B1**
(45) Date of publication and mention of the grant of the patent: **22.04.2026**
(21) Application number: 20734038.1
(22) Date of filing: 24.06.2020
(51) Int. Cl.: H01F 1/44

(54) **FERROFLUID SYSTEM CONTAINING GOLD PARTICLES**
FERROFLUIDSYSTEM MIT GOLDPARTIKELN
SYSTÈME FERROFLUIDE CONTENANT DES PARTICULES D'OR

(30) Priority: 23.07.2019 EP 19187703
(43) Date of publication of application: 01.06.2022
(73) Proprietor: Richemont International SA, 1752 Villars-sur-Glâne (CH)
(72) Inventor: MARKOVIC MILOSEVIC, Irena, 1024 ECUBLENS (CH); STUER, Michael, 2000 NEUCHÂTEL (CH); KRALJ, Slavko, 1000 LJUBLJANA (SI); MAKOVEC, Darko, 1000 LJUBLJANA (SI)
(74) Representative: Ipsilon
(86) International application number: PCT/EP2020/067754
(87) International publication number: WO 2021/013461

(56) References cited:
- EP-A1- 1 936 378
- WO-A1-2019/069990
- US-A- 5 769 996
- US-A1- 2017 316 724

## Description

### FIELD OF THE INVENTION

The invention relates to a ferrofluid system comprising a ferrofluid, gold particles and a second fluid. This composition may be used in the field of horology.

### BACKGROUND OF THE INVENTION

Depending on the intended technological field, particles may require specific properties and therefore a specific assembly or specific formulation.

For instance, US 2016/0250612 discloses encapsulated particles having a core and a silica based and aluminum containing shell.

US 2013/0040292 teaches a nanoparticle biosensor having a magnetic core, a silica layer and an outer metal shell. The core material is made of cobalt ferrite. Peptide nucleic acid is immobilized onto the outer metal shell.

US 2017/316724 discloses a magnetic fluid composite containing water, an oily magnetic fluid and poorly magnetic light shielding pieces having hydrophilic portions. Some applications require that magnetic particles move, like a fluid, in the presence of a magnetic field. In that case, the magnetic particles are conditioned in a ferrofluid.

A ferrofluid may be used in a variety of different fields. For instance, US 2004/0195540 discloses ferrofluids and their use as liquids seals. These oil based ferrofluids have an improved stability over time due to the presence of an elemental modifier that prevents or delays the aging of the magnetic particles.

US 2018/0019049 teaches a deformable inductor having a liquid magnetic core within an elastomer body. The liquid magnetic core may be a ferrofluid made of a dispersion of magnetic particles in a viscous carrier liquid.

US 2010/0277820 discloses a ferrofluid comprising a suspension of magnetic iron particles in a polar carrier, for instance ethylene glycol. The magnetic iron particles are functionalized with ligands and coated with a reflective layer.

US 4,604,222 teaches a water free ferrofluid composed of magnetic particles, an organic liquid carrier, a dispersing agent and a cationic surfactant.

US 2015/0320889 teaches an oil in water emulsion comprising nanodroplets of an oil phase containing iron magnetic particles. Surfactants stabilize these nanodroplets in water.

WO 2017/103508 also teaches an oil in water emulsion having surfactants and oil droplets containing magnetic particles.

US 2017/316724 discloses a magnetic fluid composite comprising water, an oily magnetic fluid and poorly magnetic light shielding pieces.

The poorly magnetic pieces of US 2017/316724 consist in multilayer laminates of hydrophilic layers/light shielding layers/hydrophilic layers. They can form a stable water/oil interface due to the hydrophilic layers that also require a certain degree of affinity to oil. These pieces are not functionalized through chemical interactions with a hydrophilic compound and with a hydrophobic compound.

Typically, compositions comprising an oil phase and a water phase, such as the above oil in water emulsions, are stabilized by surfactants, which prevent the coalescence of the droplets containing the magnetic particles.

Although the above ferrofluids may exhibit satisfactory properties, they are not necessarily adapted for a purpose that differs from their original technical field.

Indeed, adding pigments to ferrofluids generally afford unstable compositions. These compositions may also be subject to irreversible pigment leaching. Upon leaching, the pigments stick to the recipient containing the ferrofluid while the color of the ferrofluid turns to black i.e. the color of the magnetic particles.

Therefore, there is still a need for new ferrofluid compositions that are suitable for decorative applications. The Applicant has developed a stable ferrofluid composition that looks like a drop of liquid gold.

### SUMMARY OF THE INVENTION

The invention relates to a ferrofluid system containing magnetic particles as well as gold particles and a second fluid. This ferrofluid system has a phase having the color of gold.

More specifically, the invention relates to a ferrofluid system comprising:
a) a first phase comprising magnetic particles dispersed in a first fluid F1,
b) a second phase comprising a second fluid F2,
c) an interface layer comprising gold particles,

wherein the first fluid F1 and the second fluid F2 are not miscible,
and wherein the gold particles are functionalized with a compound (SF1) soluble in the first fluid F1 and with a compound (SF2) soluble in the second fluid F2.

This composition comprises two main phases having an interface corresponding to the intermediate layer of gold particles located between the first phase and the second phase.

The first phase is actually a ferrofluid since it comprises magnetic particles dispersed in a fluid.

The composition comprises two fluids that are not miscible. One of the fluid is hydrophilic while the other fluid is hydrophobic. However, the ferrofluid of the composition is preferably either hydrophilic or hydrophobic fluid. The ferrofluid cannot be composed of hydrophilic and hydrophobic fluids. The ferrofluid system may relate to an emulsion when one of the phases is hydrophilic and the other one is hydrophobic.

A hydrophobic fluid is not miscible with hydrophilic fluid as they form two distinct phases when mixed together.

This ferrofluid system remains stable over time. The stability of the ferrofluid system relates to the absence of any color change and/or any gold particle migration outside of the interface layer. Typically, the composition according to the invention remains stable at 25 °C for over several years, even after being shaken regularly.

The first phase is a ferrofluid. It behaves like a liquid. It can be immobilized (held in space) in the presence of a magnetic field. It can also be displaced as it follows the applied magnetic field.

The magnetic particles of the ferrofluid are ferromagnetic and/or ferrimagnetic particles, more preferably superparamagnetic particles. For instance, they may be particles containing elements such as iron, nickel or cobalt. They are preferably selected from the group consisting of iron oxide (for instance Fe₃O₄ or Fe₂O₃), cobalt iron oxide (for instance CoFe₂O₄), manganese iron oxide (for instance MnFe₂O₄), manganese zinc iron oxide (for instance (Mn,Zn)Fe₂O₄), nickel iron oxide (for instance NiFe₂O₄), and mixtures thereof.

They are preferably iron oxide particles, more preferably γ-Fe₂O₃ particles.

They can have any shape. In particular, they can be spherical, spheroidal, ellipsoidal, cubic, parallelepipedic or cylindrical (rod like).

The magnetic particles have a size preferably ranging from 2 nm to 5 µm, more preferably from 5 nm to 25 nm, for instance about 10 nm.

Typically, the size of an entity refers to the largest dimension of said entity, for instance the diameter of spherical particles or the length of parallelepipedic particles.

According to a particular embodiment, the magnetic particles represent from 0.1 to 80 wt% of the first phase, preferably from 2 to 30 wt%. According to another embodiment, it may range from 2 to 15 wt%.

The magnetic particles may be functionalized with a stabilizing agent. This stabilizing agent is preferably selected from the group consisting of molecules containing one or more of the following: carboxyl-, catechol-, amino-, sulfur-, oxygen- and phosphorus-. For instance, it may be 2-hydroxypropane-1,2,3-tricarboxylic acid i.e. citric acid (CAS Number: 77-92-9).

It helps stabilizing the magnetic particles within the volume of the first phase. It enhances the stability of the suspension of magnetic particles in the first fluid F1. It is usually bound to the magnetic particles by any one of chemical bond, non-covalent interaction, for instance hydrogen bond and coordination bond, biophysical or physical interaction, for instance biotin-avidin or electrostatic interaction.

According to a particular embodiment, the stabilizing agent represents from 0.01 to 50 wt% of the first phase, preferably from 0.1 to 4.0 wt%, more preferably from 0.2 to 4.0 wt%.

The ferrofluid has a magnetic particles / stabilizing agent weight ratio that preferably ranges from 1 / 200 to 8000 / 1, more preferably from 100 / 1 to 4 / 1.

The first phase comprising the F1 fluid of the ferrofluid system is in contact with the second phase comprising the F2 fluid through the interface layer, which comprises gold particles. The gold particles are preferably plate-like particles and give a golden color to the first phase. They are made of gold having a purity that is 14 carats or more. They may be made of 18 carat gold, 22 carat gold or even 24 carat gold. Preferably, gold is yellow gold, but white gold and red gold can also be considered.

Gold particles occupy preferably from 30 to 100 % of the area of the interface layer between the first phase and the second phase, more preferably from 95 to 100 %. Even though gold particles may overlap, the skilled person in the art will be able to adjust the quantity of gold particles depending on the volume of the first phase and/or the expected coverage.

The weight of the gold particles includes the functionalizing SF1 and SF2 molecules.

The gold particles are preferably anisotropic by shape.

These gold particles have preferably a plate-like shape, i.e., microplatelets or nanoplatelets. They may be a mix of particles having different shapes. For instance, they may be a mix of microplatelets and/or nanoplatelets including a minor amount of spherical gold particles, preferably of spherical particles having a submicron size.

Nevertheless, according to a particular embodiment, the gold particles are preferably free of spherical particles.

The gold particles have a size preferably ranging from 80 nm to 120 µm, more preferably from 0.5 µm to 80 µm, and even more preferably from 1 µm to 30 µm. As already mentioned, the size refers to the largest dimension of said particles e.g. the length, the diameter... depending on the shape of the particles.

They have a thickness that ranges from 5 nm to 80 nm, preferably from 10 nm to 80 nm, and more preferably from 20 nm to 80 nm.

The size and the thickness of the gold particles, preferably microplatelets and/or nanoplatelets, do not include the functionalizing SF1 and SF2 molecules. However, in general, the size and the thickness of the functionalized gold particles are within the ranges mentioned for the gold particles.

In general, the gold particles, preferably microplatelets and/or nanoplatelets, are functionalized through chemical interactions. They preferably form non-covalent interactions with the molecules of SF1 and SF2 such as thiol-gold interaction and/or amine-gold interaction. Accordingly, both SF1 and SF2 compounds have preferably one or more -SH and/or -NH and/or -NH₂ functional groups. Thiol functional groups have usually a greater affinity to gold particles than amine functional groups.

Accordingly, the functionalized gold particles of the ferrofluid cannot be compared to multilayer particles since the SF1 functionalizing and the SF2 functionalizing are not coating layers.

The functionalized gold particles are free of any coating, for instance free of resin films (thermoplastic resins such as polyolefin, polyamide, polyimide, polycarbonate, ethylene-vinyl acetate copolymer, ethylene-methacrylate copolymer or polyethylene terephthalate).

One of the functionalizing compounds of the gold particles is hydrophilic. It therefore affords oil in water surfactant properties to the gold particles. It preferably contains one or more OH groups and/or other polar moieties so as to improve its hydrophilic properties. It is preferably selected from the group consisting of one or more sulfur-, oxygen-, nitrogen- containing water soluble molecules. It is preferably thiocarbohydrate, for instance 2,3,4,5,6-pentahydroxy-N-(2-sulfanylethyl)hexanamide or other molecules such as compounds corresponding to any one of the following CAS numbers: 60-24-2; 1068-47-9, 19721-22-3; 59-52-9. This functionalizing compound is soluble in a hydrophilic fluid, preferably water. This compound may be the SF1 compound when the F1 fluid is hydrophilic. It may be the SF2 compound when the F2 fluid is hydrophilic.

The other functionalizing compound of the gold particles is hydrophobic. It therefore affords water in oil surfactant properties to the gold particles. It preferably contains one or more hydrocarbon chain, for instance -(CH₂-CH₂)ₙ- with n ranging from 2 to 12 and/or cyclic compound part(s), so as to improve its hydrophobic properties. It is preferably selected from the group consisting of alkyl thiols and other hydrophobic thiol-containing molecules, for instance any one of CH₃(CH₂)ₙSH with n ranging from 5 to 17 (for instance 1-dodecanethiol (CAS 112-55-0)) and other molecules such as molecules having one of the following CAS numbers: 108-98-5; 1455-21-6; 2917-26-2; 626-04-0; 1569-69-3; 13333-97-6; 100-53-8; 771-62-0; 769-40-4; 1996-44-7; 371-42-6; 2885-00-9. This functionalizing compound is soluble in a hydrophobic fluid, preferably a mineral oil or a silicone oil. This compound may be the SF1 compound when the F1 fluid is hydrophobic. It may be the SF2 compound when the F2 fluid is hydrophobic.

In view of the properties of the gold particles, the ferrofluid system is preferably free of surfactants, such as sorbitan or oleate based surfactants.

The SF1 is soluble in the first fluid as 1 mass part of SF1 readily dissolves in 30 mass parts of first fluid, at 25 °C.

Since the gold particles are not soluble in the first fluid and in the second fluid, the SF1 and the SF2 compounds anchor gold particles on the interface between hydrophilic and hydrophobic fluid.

For instance, when the first fluid is a hydrophilic fluid and the second fluid is a hydrophobic fluid, the SF1 anchors the gold particles to the hydrophilic fluid while the SF2 anchors the gold particles to the hydrophobic fluid. When the first fluid is a hydrophobic fluid and the second fluid is a hydrophilic fluid, the SF1 anchors the gold particles to the hydrophobic fluid while the SF2 anchors the gold particles to the hydrophilic fluid.

Typically, the ferrofluid system contains a hydrophobic fluid and a hydrophilic fluid that are not miscible.

The hydrophobic fluid is preferably an oil, e.g. a mineral oil or a silicon oil. For instance, it may be selected from the group consisting of C₅-C₂₄ alkanes, C₅-C₂₄ cyclic hydrocarbon compounds, silicone oils, organohalides such as organochlorides and organofluorines. It is preferably selected from the group consisting of higher alkanes (C₁₀ and above). Typically, oils comprise a mixture of compounds, for instance light oils may comprise a mixture of C₅-C₉ alkanes.

The hydrophilic fluid is preferably selected from the group consisting of water; DMSO (dimethyl sulfoxide); DMF (dimethylformamide); glycols such as ethylene glycol; alcohols such as methanol, ethanol; and others. Most preferably, the hydrophilic fluid is water.

The SF2 is soluble in the second fluid as 1 mass part of SF2 readily dissolves in 30 mass parts of second fluid, at 25 °C. Nevertheless, the second fluid may also be air or another gas, for instance nitrogen or a noble gas, preferably argon or helium.

Due to the presence of both SF1 and SF2, the gold particles are at the interface between the first phase and the second phase.

The gold particles have a SF1 / SF2 weight ratio of preferably between 1 / 15 and 15 / 1, more preferably between 1 / 10 and 10 / 1, and even more preferably between 1 / 3 and 3/1.

Furthermore, according to a particular embodiment, the SF1 represent from 0.01 to 30 wt% by weight of the gold particles (preferably microplatelets and/or nanoplatelets), preferably 0.1 to 20 wt%, more preferably 2 to 10 wt%.

According to another particular embodiment, the SF2 represent from 0.01 to 30 wt% by weight of the gold particles (preferably microplatelets and/or nanoplatelets), preferably 0.1 to 20 wt%, more preferably 2 to 10 wt%.

In summary, the first phase comprises a suspension containing magnetic particles and, preferably, at least one stabilizing agent.

The ferrofluid system also comprises a second phase based on a second fluid F2 that is not miscible with the first fluid F1.

The interface is comprised by SF1 and SF2 functionalized gold particles.

According to a particular embodiment, the ferrofluid system can have any first phase / second phase volume ratio between 1 / 3 and 1 / 20.

The first phase has a volume that preferably range from 50 µL to 50 mL.

The first phase preferably defines a single volume that is located within the second phase. It is not an emulsion comprising a plurality of drops of a first phase dispersed in a second phase. Consequently, the ferrofluid system of the invention is preferably free of non-attached SF1 and/or SF2 stabilizing agents. The SF1 and SF2 molecules of the ferrofluid system are preferably all attached to the gold particles.

According to a particular embodiment, the ferrofluid system comprises:
a) a first phase comprising magnetic particles dispersed in a first fluid F1, wherein F1 is a hydrophilic fluid, preferably water,
b) a second phase comprising a second fluid F2, wherein F2 is a hydrophobic fluid preferably selected from the group consisting of alkanes, cyclic hydrocarbon compounds, silicone oils, mineral oils, and organohalides,
c) an interface layer comprising SF 1- and SF2-functionalized gold particles.

According to another particular embodiment, the ferrofluid system comprises:
a) a first phase comprising magnetic particles dispersed in a first fluid F1, wherein F1 is a hydrophobic fluid preferably selected from the group consisting of alkanes, cyclic hydrocarbon compounds, silicone oils, mineral oils, and organohalides,
b) a second phase comprising a second fluid F2, wherein F2 is a hydrophilic fluid, preferably water.
c) an interface layer comprising SF1- and SF2-functionalized gold particles.

The invention also relates to the use of the ferrofluid system in the field of horology, for instance a timepiece comprising this ferrofluid system. For instance, it can afford aesthetic properties as it provides a visual display that behaves like a moving fluid in the presence of a magnetic field.

The invention also relates to a method for preparing the above described ferrofluid system according to the following steps:
1/ a suspension of magnetic particles is prepared as a first fluid F1,
2/ SF1 and SF2 functionalized gold particles are added to first fluid F1,
3/ the resulting composition is mixed with a second fluid F2.

As already mentioned, the magnetic particles may be functionalized with a stabilizing agent, for instance citric acid.

The gold particles may be prepared by reduction of auric salt, preferably HAuCl₄. The reduction may preferably be carried out in the presence of compounds such as aniline and ethylene glycol.

The gold particles can be functionalized by the SF1 and the SF2 sequentially according to conventional reactions that are within the knowledge of the skilled person in the art. Indeed, the SF1 functionalization is preferably carried out in the F1 fluid or a solvent in which the SF1 compound is soluble while the SF2 functionalization is preferably first carried out in the F2 fluid or a solvent in which the SF2 compound is soluble. The order of functionalization (SF1 or SF2 at first) is not important. The SF1 and/or the SF2 functionalization(s) may also be carried out in the presence of the magnetic particles.

Steps 1/ through 3/ may be carried out at a temperature of between 0 °C and 90 °C, preferably above 15 °C.

The invention and its advantages will become more apparent to one skilled in the art from the following figures.

### BRIEF DESCRIPTION OF THE DRAWINGS

Figure 1 illustrates the first phase of the ferrofluid system according to the invention.
Figure 2 is a photography of the ferrofluid system according to the invention.

### DETAILED DESCRIPTION OF EMBODIMENTS OF THE INVENTION

The ferrofluid system has a first phase comprising magnetic particles and the second phase which is not miscible with the first one while an interface is occupied with gold particles. Figure 1 illustrate the first phase in which the magnetic particles (1) are dispersed in the fluid F1 (2).

The interface layer (3) comprises gold particles (4) (preferably microplatelets and/or nanoplatelets) that are functionalized with the SF1 and SF2 compounds.

Thanks to the SF1 and to the SF2, the gold particles (4) decorate an interface between the suspension of magnetic particles (1) and the second phase that comprises the second fluid in which the first fluid is not miscible.

However, the gold particles (4) do not act as a stabilizing agent since the gold particles do not prevent droplets of the first fluid F1 from collapsing together.

## Claims

1. Ferrofluid system **characterized in that** it comprises:
a) a first phase comprising magnetic particles dispersed in a first fluid F1,
b) a second phase comprising a second fluid F2,
c) an interface layer comprising gold particles made of gold having a purity that is 14 carats or more and having a thickness ranging from 5 nm to 80 nm,
wherein the first fluid F1 and the second fluid F2 are not miscible,
wherein the gold particles are functionalized with a compound (SF1) soluble in the first fluid F1 and with a compound (SF2) soluble in the second fluid F2,
wherein one of the functionalizing compounds of the gold particles is hydrophilic while the other functionalizing compound of the gold particles is hydrophobic,
one of the fluids is hydrophilic while the other fluid is hydrophobic, and
wherein the functionalized gold particles are free of any coating.

2. Ferrofluid system according to claim 1, ***characterized* in that** the magnetic particles are iron oxide particles, preferably γ-Fe₂O₃ particles.

3. Ferrofluid system according to any one of claims 1 to 2, ***characterized* in that** the magnetic particles have a size ranging from 2 nm to 5 µm, preferably from 5 nm to 25 nm.

4. Ferrofluid system according to any one of claims 1 to 3, ***characterized* in that** the magnetic particles are functionalized with a stabilizing agent that is selected from the group consisting molecules containing one or more of carboxyl-, catechol-, amino-, sulfur-, oxygen- and phosphorus-, preferably 2-hydroxypropane-1,2,3-tricarboxylic acid.

5. Ferrofluid system according to any one of claims 1 to 4, ***characterized* in that** the gold particles occupy from 30 % to 100 % of the area of interface layer between the first phase and the second phase.

6. Ferrofluid system according to any one of claims 1 to 5, ***characterized* in that** the gold particles have a size ranging from 80 nm to 120 µm, preferably from 0.5 µm to 80 µm, more preferably from 1 µm to 30 µm.

7. Ferrofluid system according to any one of claims 1 to 6, ***characterized* in that** the gold particles have a thickness ranging from 10 nm to 80 nm, preferably from 20 nm to 80 nm.

8. Ferrofluid system according to any one of claims 1 to 7, ***characterized* in that** the first fluid F1 is hydrophilic, preferably water, and **in that** the SF1 compound is selected from the group consisting of one or more sulfur-, oxygen-, nitrogen- containing water soluble molecules, preferably any one of 2,3,4,5,6-pentahydroxy-N-(2-sulfanylethyl)hexanamide and any one of the following molecules: 2-mercaptoethanol of CAS number 60-24-2; 1-mercapto-2-propanol of CAS number 1068-47-9; 3-mercapto-1-propanol of CAS number 19721-22-3 and 2,3-dimercapto-1-propanol of CAS number 59-52-9.

9. Ferrofluid system according to any one of claims 1 to 8, ***characterized* in that** the second fluid F2 is hydrophobic and **in that** the SF2 compound is selected from the group of alkyl thiols and other hydrophobic thiol-containing molecules, preferably any one of 1-dodecanethiol and one of the following molecules: thiophenol of CAS number 108-98-5; 1-nonanethiol of CAS number 1455-21-6; hexadecanethiol of CAS number 2917-26-2; 1,3-benzenedithiol of CAS number 626-04-0; cyclohexanethiol of CAS number 1569-69-3; 2-(trifluoromethyl)benzenethiol of CAS number 13333-97-6; benzyl mercaptan of CAS number 100-53-8; pentafluorobenzenethiol of CAS number 771-62-0; 2,3,5,6-tetrafluorothiophenol of CAS number 769-40-4; 2,4-difluorothiophenol of CAS number 1996-44-7; 4-fluorobenzenethiol of CAS number 371-42-6; and 1-octadecanethiol of CAS number 2885-00-9.

10. Ferrofluid system according to any one of claims 1 to 9, ***characterized* in that** the gold particles have a SF1 / SF2 weight ratio of between 1 / 15 and 15 / 1, preferably between 1 / 10 and 10 / 1, and more preferably between 1 / 3 and 3 / 1.

11. Ferrofluid system according to any one of claims 1 to 10, ***characterized* in that** the ferrofluid system has any first phase / second phase volume ratio between 1 / 3 and 1 / 20.

12. Ferrofluid system according to any one of claims 1 to 11, ***characterized* in that** the first fluid F1 is a hydrophilic fluid, preferably water, and **in that** the second fluid F2 is a hydrophobic fluid, preferably selected from the group consisting of alkanes, cyclic hydrocarbon compounds, silicone oils, mineral oils, and organohalides.

13. Ferrofluid system according to any one of claims 1 to 7, ***characterized* in that** the first fluid F1 is hydrophobic, and the SF1 compound is selected from the group of alkyl thiols and other hydrophobic thiol-containing molecules, preferably any one of 1-dodecanethiol and one of the following molecules: thiophenol of CAS number 108-98-5; 1-nonanethiol of CAS number 1455-21-6; hexadecanethiol of CAS number 2917-26-2; 1,3-benzenedithiol of CAS number 626-04-0; cyclohexanethiol of CAS number 1569-69-3; 2-(trifluoromethyl)benzenethiol of CAS number 13333-97-6; benzyl mercaptan of CAS number 100-53-8; pentafluorobenzenethiol of CAS number 771-62-0; 2,3,5,6-tetrafluorothiophenol of CAS number 769-40-4; 2,4-difluorothiophenol of CAS number 1996-44-7; 4-fluorobenzenethiol of CAS number 371-42-6; and 1-octadecanethiol of CAS number 2885-00-9,
and wherein the second fluid F2 is hydrophilic, preferably water, and the SF2 compound is selected from the group consisting of one or more sulfur-, oxygen-, nitrogen-containing water soluble molecules, preferably any one of 2,3,4,5,6-pentahydroxy-N-(2-sulfanylethyl)hexanamide and any one of the following molecules: 2-mercaptoethanol of CAS number 60-24-2; 1-mercapto-2-propanol of CAS number 1068-47-9; 3-mercapto-1-propanol of CAS number 19721-22-3 and 2,3-dimercapto-1-propanol of CAS number 59-52-9.

14. Ferrofluid system according to any one of claims 1 to 13, ***characterized* in that** the first phase defines a single volume that is within the second phase, and **in that** the gold particles are nanoplatelets functionalized through chemical interactions with the SF1 and SF2 compounds.

15. Use of a ferrofluid system in the field of horology, **characterized in that** the ferrofluid system is the ferrofluid system according to any one of claims 1 to 14.

## Patentansprüche

1. Ferrofluid-System, ***dadurch gekennzeichnet, dass*** es Folgendes umfasst:
a) eine erste Phase, die magnetische Partikel umfasst, welche in einem ersten Fluid F1 dispergiert sind,
b) eine zweite Phase, die ein zweites Fluid F2 umfasst,
c) einer Grenzflächenschicht, die Goldpartikel umfasst, welche aus Gold hergestellt sind, dessen Reinheit von mindestens 14 Karat beträgt, und die eine Dicke im Bereich von 5 nm bis 80 nm aufweist,
wobei das erste Fluid F1 und das zweite Fluid F2 nicht mischbar sind,
wobei die Goldpartikel mit einer Verbindung (SF1), die in dem ersten Fluid F1 löslich ist, und mit einer Verbindung (SF2), die in dem zweiten Fluid F2 löslich ist, funktionalisiert sind,
wobei eine der funktionalisierenden Verbindungen der Goldpartikel hydrophil ist, während die andere funktionalisierende Verbindung der Goldpartikel hydrophob ist, eines der Fluids hydrophil ist, während das andere Fluid hydrophob ist, und
wobei die funktionalisierten Goldpartikel frei von jedweder Beschichtung sind.

2. Ferrofluid-System gemäß Anspruch 1, ***dadurch gekennzeichnet, dass*** es sich bei den magnetischen Partikeln um Eisenoxidpartikel, vorzugsweise γ-Fe₂O₃ Partikel, handelt.

3. Ferrofluid-System gemäß einem beliebigen der Ansprüche 1 bis 2, ***dadurch gekennzeichnet, dass*** die magnetischen Partikel eine Größe von 2 nm bis 5 µm, vorzugsweise von 5 nm bis 25 nm aufweisen.

4. Ferrofluidsystem gemäß einem beliebigen der Ansprüche 1 bis 3, ***dadurch gekennzeichnet, dass*** die magnetischen Partikel mit einem Stabilisierungsmittel funktionalisiert sind, das aus der Gruppe ausgewählt, welche aus Molekülen besteht, die eines oder mehrere von Carboxyl, Brenzcatechin, Amino, Schwefel, Sauerstoff und Phosphor enthalten, wobei es sich vorzugsweise um 2-Hydroxypropan-1,2,3-tricarbonsäure handelt.

5. Ferrofluid-System gemäß einem beliebigen der Ansprüche 1 bis 4, ***dadurch gekennzeichnet, dass*** die Goldpartikel 30 % bis 100 % der Fläche der Grenzflächenschicht zwischen der ersten Phase und der zweiten Phase einnehmen.

6. Ferrofluid-System gemäß einem beliebigen der Ansprüche 1 bis 5, ***dadurch gekennzeichnet, dass*** die Goldpartikel eine Größe im Bereich von 80 nm bis 120 µm, vorzugsweise von 0,5 µm bis 80 µm, insbesondere von 1 µm bis 30 µm aufweisen.

7. Ferrofluid-System gemäß einem beliebigen der Ansprüche 1 bis 6, ***dadurch gekennzeichnet, dass*** die Goldpartikel eine Dicke von 10 nm bis 80 nm, vorzugsweise von 20 nm bis 80 nm aufweisen.

8. Ferrofluid-System gemäß einem beliebigen der Ansprüche 1 bis 7, ***dadurch gekennzeichnet, dass*** das erste Fluid F1 hydrophil ist, wobei es sich vorzugsweise um Wasser handelt, und dadurch, dass die SF1-Verbindung aus der Gruppe ausgewählt ist, die aus einem oder mehreren schwefel-, sauerstoff-, stickstoffhaltigen wasserlöslichen Molekülen besteht, wobei es sich vorzugsweise um ein beliebiges von 2,3,4,5,6-Pentahydroxy-N-(2-sulfanylethyl)hexanamid und einem beliebigen der folgenden Moleküle handelt: 2-Mercaptoethanol mit der CAS-Nummer 60-24-2; 1-Mercapto-2-propanol mit der CAS-Nummer 1068-47-9; 3-Mercapto-1-propanol mit der CAS-Nummer 19721-22-3 und 2,3-Dimercapto-1-propanol mit der CAS-Nummer 59-52-9.

9. Ferrofluid-System gemäß einem beliebigen der Ansprüche 1 bis 8, ***dadurch gekennzeichnet, dass*** das zweite Fluid F2 hydrophob ist und dass die SF2-Verbindung aus der Gruppe der Alkylthiole und anderer hydrophober thiolhaltiger Moleküle ausgewählt ist, wobei es sich vorzugsweise um ein beliebiges von 1-Dodecanthiol und einem der folgenden Moleküle handelt: Thiophenol mit der CAS-Nummer 108-98-5; 1-Nonanthiol mit der CAS-Nummer 1455-21-6; Hexadecanthiol mit der CAS-Nummer 2917-26-2; 1,3-Benzoldithiol mit der CAS-Nummer 626-04-0; Cyclohexanthiol mit der CAS-Nummer 1569-69-3; 2-(Trifluormethyl)benzolthiol mit der CAS-Nummer 13333-97-6; Benzylmercaptan mit der CAS-Nummer 100-53-8; Pentafluorbenzolthiol mit der CAS-Nummer 771-62-0; 2,3,5,6-Tetrafluorthiophenol mit der CAS-Nummer 769-40-4; 2,4-Difluorthiophenol mit der CAS-Nummer 1996-44-7; 4-Fluorbenzolthiol mit der CAS-Nummer 371-42-6; und 1-Octadecanthiol mit der CAS-Nummer 2885-00-9.

10. Ferrofluid-System gemäß einem beliebigen der Ansprüche 1 bis 9, ***dadurch gekennzeichnet, dass*** die Goldpartikel ein SF1/SF2-Gewichtsverhältnis zwischen 1/15 und 15/1, vorzugsweise zwischen 1/10 und 10/1 und insbesondere zwischen 1/3 und 3/1 aufweisen.

11. Ferrofluid-System gemäß einem beliebigen der Ansprüche 1 bis 10, ***dadurch gekennzeichnet, dass*** das Ferrofluid-System ein beliebiges Volumenverhältnis der ersten Phase/zweiten Phase zwischen 1/3 und 1/20 aufweist.

12. Ferrofluid-System gemäß einem beliebigen der Ansprüche 1 bis 11, ***dadurch gekennzeichnet, dass*** das erste Fluid F1 ein hydrophiles Fluid ist, wobei es sich vorzugsweise um Wasser handelt, und dadurch, dass das zweite Fluid F2 ein hydrophobes Fluid ist, wobei es vorzugsweise aus der Gruppe ausgewählt ist, die aus Alkanen, zyklischen Kohlenwasserstoffverbindungen, Silikonölen, Mineralölen und Organohalogeniden besteht.

13. Ferrofluid-System gemäß einem beliebigen der Ansprüche 1 bis 7, ***dadurch gekennzeichnet, dass*** das erste Fluid F1 hydrophob ist und die SF1-Verbindung aus der Gruppe der Alkylthiole und anderen hydrophoben thiolhaltigen Moleküle ausgewählt ist, wobei es sich vorzugsweise um ein beliebiges von 1-Dodecanthiol und einem der folgenden Moleküle handelt: Thiophenol mit der CAS-Nummer 108-98-5; 1-Nonanthiol mit der CAS-Nummer 1455-21-6; Hexadecanthiol mit der CAS-Nummer 2917-26-2; 1,3-Benzoldithiol mit der CAS-Nummer 626-04-0; Cyclohexanthiol mit der CAS-Nummer 1569-69-3; 2-(Trifluormethyl)benzolthiol mit der CAS-Nummer 13333-97-6; Benzylmercaptan mit der CAS-Nummer 100-53-8; Pentafluorbenzolthiol mit der CAS-Nummer 771-62-0; 2,3,5,6-Tetrafluorthiophenol mit der CAS-Nummer 769-40-4; 2,4-Difluorthiophenol mit der CAS-Nummer 1996-44-7; 4-Fluorbenzolthiol mit der CAS-Nummer 371-42-6; und 1-Octadecanthiol mit der CAS-Nummer 2885-00-9,
und wobei das zweite Fluid F2 hydrophil ist, wobei es sich vorzugsweise um Wasser handelt, und die SF2-Verbindung aus der Gruppe ausgewählt ist, die aus einem oder mehreren schwefel-, sauerstoff-, stickstoffhaltigen wasserlöslichen Molekülen besteht, wobei es sich vorzugweise um ein beliebiges von 2,3,4,5,6-Pentahydroxy-N-(2-sulfanylethyl)hexanamid und einem beliebigen der folgenden Moleküle handelt: 2-Mercaptoethanol mit der CAS-Nummer 60-24-2; 1-Mercapto-2-propanol mit der CAS-Nummer 1068-47-9; 3-Mercapto-1-propanol mit der CAS-Nummer 19721-22-3 und 2,3-Dimercapto-1-propanol mit der CAS-Nummer 59-52-9.

14. Ferrofluidsystem gemäß einem beliebigen der Ansprüche 1 bis 13, ***dadurch gekennzeichnet, dass*** die erste Phase ein einziges Volumen festlegt, das sich innerhalb der zweiten Phase befindet, und dass es sich bei den Goldpartikeln um Nanoplättchen handelt, die durch chemische Wechselwirkungen mit den SF1- und SF2-Verbindungen funktionalisiert sind.

15. Verwendung eines Ferrofluid-Systems im Bereich der Uhrenindustrie, ***dadurch gekennzeichnet, dass*** es sich bei dem Ferrofluid-System um das Ferrofluid-System gemäß einem beliebigen der Ansprüche 1 bis 14 handelt.

## Revendications

1. Système de ferrofluide, **caractérisé en ce qu'**il comprend :
a) une première phase comprenant des particules magnétiques dispersées dans un premier fluide F1,
b) une seconde phase comprenant un second fluide F2,
c) une couche d'interface comprenant des particules d'or en or d'une pureté de 14 carats ou plus et d'une épaisseur allant de 5 nm à 80 nm,
dans lequel le premier fluide F1 et le second fluide F2 ne sont pas miscibles,
dans lequel les particules d'or sont fonctionnalisées avec un composé (SF1) soluble dans le premier fluide F1 et avec un composé (SF2) soluble dans le second fluide F2,
dans lequel l'un des composés de fonctionnalisation des particules d'or est hydrophile tandis que l'autre composé de fonctionnalisation des particules d'or est hydrophobe, l'un des fluides est hydrophile tandis que l'autre fluide est hydrophobe, et
dans lequel les particules d'or fonctionnalisées sont exemptes de tout revêtement.

2. Système de ferrofluide selon la revendication 1, **caractérisé en ce que** les particules magnétiques sont des particules d'oxyde de fer, de préférence des particules de γ-Fe₂O₃.

3. Système de ferrofluide selon l'une quelconque des revendications 1 à 2, **caractérisé en ce que** les particules magnétiques présentent une taille allant de 2 nm à 5 µm, de préférence de 5 nm à 25 nm.

4. Système de ferrofluide selon l'une quelconque des revendications 1 à 3, **caractérisé en ce que** les particules magnétiques sont fonctionnalisées avec un agent stabilisant qui est choisi dans le groupe comprenant des molécules contenant un ou plusieurs parmi un acide carboxyle, catéchol, amino, soufré, oxygéné et phosphoré, de préférence un acide 2-hydroxypropane-1,2,3-tricarboxylique.

5. Système de ferrofluide selon l'une quelconque des revendications 1 à 4, **caractérisé en ce que** les particules d'or occupent de 30 % à 100 % de la surface de couche d'interface entre la première phase et la seconde phase.

6. Système de ferrofluide selon l'une quelconque des revendications 1 à 5, **caractérisé en ce que** les particules d'or présentent une taille allant de 80 nm à 120 µm, de préférence de 0,5 µm à 80 µm, de manière plus préférée de 1 µm à 30 µm.

7. Système de ferrofluide selon l'une quelconque des revendications 1 à 6, **caractérisé en ce que** les particules d'or présentent une épaisseur allant de 10 nm à 80 nm, de préférence de 20 nm à 80 nm.

8. Système de ferrofluide selon l'une quelconque des revendications 1 à 7, **caractérisé en ce que** le premier fluide F1 est hydrophile, de préférence de l'eau, et **en ce que** le composé SF1 est choisi dans le groupe comprenant une ou plusieurs molécules solubles dans l'eau contenant du soufre, de l'oxygène, de l'azote, de préférence l'une quelconque de 2,3,4,5,6-pentahydroxy-N- (2-sulfanyléthyl)hexanamide et l'une quelconque des molécules suivantes : 2-mercaptoéthanol, numéro CAS 60-24-2 ; 1-mercapto-2-propanol, numéro CAS 1068-47-9 ; 3-mercapto-1-propanol, numéro CAS 19721-22-3 et 2,3-dimercapto-1-propanol, numéro CAS 59-52-9.

9. Système de ferrofluide selon l'une quelconque des revendications 1 à 8, **caractérisé en ce que** le second fluide F2 est hydrophobe et **en ce que** le composé SF2 est choisi dans le groupe comprenant des alkylthiols et d'autres molécules hydrophobes contenant du thiol, de préférence un quelconque parmi le 1-dodécanethiol et l'une des molécules suivantes : thiophénol, numéro CAS 108-98-5 ; 1-nonanethiol, numéro CAS 1455-21-6 ; hexadécanethiol, numéro CAS 2917-26-2 ; 1,3-benzènedithiol, numéro CAS 626-04-0 ; cyclohexanethiol, numéro CAS 1569-69-3 ; 2-(trifluorométhyl)benzènethiol, numéro CAS 13333-97-6 ; benzyl mercaptan, numéro CAS 100-53-8 ; pentafluorobenzènethiol, numéro CAS 771-62-0 ; 2,3,5,6-tétrafluorothiophénol, numéro CAS 769-40-4 ; 2,4-difluorothiophénol, numéro CAS 1996-44-7 ; 4-fluorobenzènethiol, numéro CAS 371-42-6 ; et 1-octadécanethiol, numéro CAS 28-0085-9.

10. Système de ferrofluide selon l'une quelconque des revendications 1 à 9, **caractérisé en ce que** les particules d'or présentant un rapport pondéral SF1/SF2 compris entre 1/15 et 15/1, de préférence entre 1/10 et 10/1, et plus préférentiellement entre 1/3 et 3/1.

11. Système de ferrofluide selon l'une quelconque des revendications 1 à 10, **caractérisé en ce que** le système de ferrofluide a un rapport de volume de première phase/seconde phase quelconque compris entre 1/3 et 1/20.

12. Système de ferrofluide selon l'une quelconque des revendications 1 à 11, **caractérisé en ce que** le premier fluide F1 est un fluide hydrophile, de préférence de l'eau, et **en ce que** le second fluide F2 est un fluide hydrophobe, de préférence choisi dans le groupe constitué par des alcanes, des composés hydrocarbonés cycliques, des huiles de silicone, des huiles minérales et des organohalogénures.

13. Système de ferrofluide selon l'une quelconque des revendications 1 à 7, **caractérisé en ce que** le premier fluide F1 est hydrophobe, et le composé SF1 est choisi dans le groupe comprenant des alkylthiols et d'autres molécules hydrophobes contenant du thiol, de préférence l'un quelconque parmi le 1-dodécanethiol et l'une des molécules suivantes : thiophénol, numéro CAS 108-98-5 ; 1-nonanethiol, numéro CAS 1455-21-6 ; hexadécanethiol, numéro CAS 2917-26-2 ; 1,3-benzènedithiol, numéro CAS 626-04-0 ; cyclohexanethiol, numéro CAS 1569-69-3 ; 2-(trifluorométhyl)benzènethiol, numéro CAS 13333-97-6 ; benzyl mercaptan, numéro CAS 100-53-8 ; pentafluorobenzènethiol, numéro CAS 771-62-0 ; 2,3,5,6-tétrafluorothiophénol, numéro CAS 769-40-4 ; 2,4-difluorothiophénol, numéro CAS 1996-44-7 ; 4-fluorobenzènethiol, numéro CAS 371-42-6 ; et 1-octadécanethiol de numéro CAS 2885-00-9, et le second fluide dans lequel F2 est hydrophile, de préférence de l'eau, et le composé SF2 est choisi dans le groupe constitué par une ou plusieurs molécules contenant du soufre, de l'oxygène, de l'azote, de préférence une quelconque parmi 2,3,4,5-pentahydroxylthanyamide et l'une quelconque des molécules suivantes : 2-mercaptoéthanol, numéro CAS 60-24-2 ; 1-mercapto-2-propanol, numéro CAS 1068-47-9 ; 3-mercapto-1-propanol, numéro CAS 19721-22-3 et 2,3-dimercapto-1-propanol, numéro CAS 59-52-9.

14. Système de ferrofluide selon l'une quelconque des revendications 1 à 13, **caractérisé en ce que** la première phase définit un volume unique qui se trouve dans la seconde phase, et **en ce que** les particules d'or sont des nanoplaquettes fonctionnalisées par des interactions chimiques avec les composés SF1 et SF2.

15. Utilisation d'un système de ferrofluide dans le domaine de l'horlogerie, **caractérisé en ce que** le système de ferrofluide est le système de ferrofluide selon l'une quelconque des revendications 1 à 14.
